

Patented Sept. 23, 1947

2,427,966

## UNITED STATES PATENT OFFICE

2,427,966

WELDING ELECTRODE COATING  
COMPOSITION

Carl Jonathan Hirschler, New Malden, and William George Campbell, Aylesbury, England

No Drawing. Application November 13, 1944,  
Serial No. 563,318. In Great Britain November  
16, 1943

2 Claims. (Cl. 219—8)

**1** This invention relates to cellulosic material and to welding electrode coating compositions containing the same and welding electrodes coated with such compositions.

As at present manufactured the coating of shielded welding electrodes contains as an important ingredient cotton flock or other form of comminuted cellulose.

One object of the present invention is the production of a cellulosic material which can be used with advantage in the coating of welding electrodes in substitution for a part or the whole of the flock or other form of cellulose which hitherto has been used for this purpose, further objects being the production of coating compositions for electrodes and electrodes furnished with a coating containing cellulosic material.

The invention consists in subjecting wood flour or other suitably comminuted lignin containing cellulosic material to acid hydrolysis, washing the hydrolysed product and drying and grinding the residual material of higher lignin content to a desired average particle size.

In this way a product is obtained which is of a fibrous character and contains a higher proportion of lignin and thus a smaller proportion of cellulose than the lignified material treated, which it will be appreciated is of advantage from the point of view of the use of the material in electrode coating compositions, as it is known that the pyrolysis of cellulose gives rise to acrid fumes which are particularly objectionable when shielded welding electrodes are used in confined spaces.

The treated material furthermore has a superior affinity toward silicate solutions which is attributable to substantially its higher lignin content.

In other words the reduction of the cellulose content of the material which is effected by the treatment in accordance with the invention has the effect of effecting a reduction in the production of acrid fumes and maintaining or increasing the extent to which a given quantity of the product can retain a silicate within the coating of the finished electrodes without depriving the product of its other desirable properties.

A coating composition in accordance with the invention consists in lignin-containing cellulosic material obtained in the manner above specified, in association with appropriate binding agents and other essential and any desirable constituents of the coating compositions previously employed for the like purpose.

The invention also consists in electrodes fur-

nished with a coating composition as defined in the preceding paragraph.

The following particulars are given by way of example to illustrate suitable methods of carrying the invention into effect:

*Example I*

10 lb. of air-dry 60-mesh spruce wood flour is incorporated with a 5 per cent. (weight/volume) aqueous solution of hydrochloric acid in the proportion of 1 gallon of solution per pound of wood flour. The mixture is boiled at atmospheric pressure for two hours.

Thereafter the solid product is isolated by filtration, washed with hot water until free from acid and dried to constant weight at 100 to 105° C. The dried product is then subjected to light grinding in an end-runner mill to give a powder capable of passing a 120-mesh screen.

15 In the treatment as above described of wood flour which was found by analysis to contain 29.2 per cent. of lignin, the finished product containing 36.3 per cent. and the complete process had the effect of lowering the absorbency towards liquid water as found by a standard testing procedure from a value of 6 ml. per gramme in the case of the original wood flour to 2.8 ml. per gramme in the finished product.

*Example II*

20 245 lb. of air-dry 10-mesh spruce sawdust containing 32 lb. of water as moisture of condition is incorporated with 148.5 gallons of water and 336 lb. of hydrochloric acid of 28° Tw. The mixture is boiled at atmospheric pressure for two hours. The solid product is thereafter isolated by filtration, washed with hot water until free from acid and dried to constant weight at 100 to 105° C.

25 The dried product is then ground to pass a 200-mesh screen or until a sample, after thorough mixing with 20 times its weight of distilled water and drainage on a filter under atmospheric pressure retains not more than three times its own weight of water.

*Example III*

30 245 lb. of air-dry 10-mesh spruce sawdust containing 32 lb. of water as moisture of condition is incorporated with 121 gallons of the spent acid liquor removed by filtration and prior to washing from a previous cook as in Example II above, 112 lb. of hydrochloric acid of 28° Tw. and 47 gallons of water. The mixture is boiled for two hours at atmospheric pressure and the solid

product isolated, dried and ground as in Example II.

We have found that in continuous production the procedure indicated in Example III may with advantage, as regards economy of acid, be followed until four batches of 245 lbs. of sawdust have been so treated. In practice lignin contents ranging from 36 per cent. up to and including 40 per cent. have been obtained.

*Example IV*

This example relates to the use of hydrochloric acid of 20 per cent. concentration, a solution from which, after use, hydrochloric acid can be recovered for re-use by distillation. 10 lbs. of air-dry 60-mesh spruce wood flour is incorporated with a 20 per cent. (weight/volume) solution of hydrochloric acid in the proportion of 0.85 gallons of solution per pound of wood flour. The mixture is boiled for two hours at atmospheric pressure in a closed vessel fitted with a reflux condenser. After removal of the spent liquor containing soluble decomposition products of the wood the solid product is washed, dried and ground as in Examples II and III above. In this way a material of 65 to 70 per cent. lignin content may be obtained.

We have found that when incorporated with sodium or potassium silicate solution of specific gravity of about 1.36 so as to form a composition of the appropriate consistency for coating welding electrodes, the air-dry product as prepared in Examples I, II and III above required, in the average, 4.69 times its own weight of sodium silicate solution. The corresponding average figure for the air-dry product prepared as in Example IV above was 6.3 and for powdered cotton cellulose of similar particle size it was 2.72.

The following is an example of a coating composition for welding electrodes within the scope of the invention:

| Per cent by weight                    |           |    |
|---------------------------------------|-----------|----|
| Titanium dioxide or rutile            | 20-40     |    |
| Ferromanganese                        | 15-25     | 45 |
| Lignin-containing cellulosic material | 30-50     |    |
| Felspar or other silicates            | Remainder |    |

To a mixture within this range of compositions there is added an appropriate proportion of a sodium or potassium silicate solution of the specific gravity above stated to yield a mass capable of being extruded.

Electrodes in accordance with the invention are produced by extrusion of the composition through a die through which also the welding electrodes are passed.

It is to be understood that our invention is in no way confined to the above examples and variations may be made. Thus both the concentration of acid and time of boiling may be varied and also the fineness of grinding of the end product and in the constitution of the coating composition.

We claim:

1. A coating composition for welding electrodes comprising ligno-cellulosic material, the lignin constituting from about 36 percent to 70 percent thereof, and a binding agent.

2. A coating composition for welding electrodes comprising ligno-cellulosic material, the lignin constituting from about 36 percent to 70 percent thereof, and an alkali metal silicate solution as a binding agent, the silicate solution amounting to between about 4.69 and 6.3 times the weight of the ligno-cellulosic material, said solution having a specific gravity of about 1.36.

CARL JONATHAN HIRSCHLER.  
WILLIAM GEORGE CAMPBELL.

REFERENCES CITED

The following references are of record in the file of this patent:

UNITED STATES PATENTS

| Number     | Name             | Date          |
|------------|------------------|---------------|
| Re. 22,295 | Olson            | Mar. 30, 1943 |
| 1,884,715  | Jerabek (1)      | Oct. 25, 1932 |
| 2,086,132  | Jerabek (2)      | July 6, 1937  |
| 2,209,829  | Rasmussen et al. | July 30, 1940 |
| 2,269,665  | Herbst           | Jan. 13, 1942 |